

## UNITED STATES PATENT OFFICE

2,087,767

CONVERSION OF IRON-CARBON ALLOYS  
INTO PRODUCTS OF SHEETED AND  
OTHER SHAPESNathan H. Schermer, Detroit, Mich., assignor to  
Stellum, Inc., Cleveland, Ohio, a corporation  
of OhioNo Drawing. Application April 17, 1936,  
Serial No. 75,014

12 Claims. (Cl. 148—12)

This invention relates in general to the treatment of cast iron-carbon alloys, particularly white cast iron, for the obtaining of products in sheeted or other shapes with tensile strength and m-  
5 chinability, corrosion resistance, etc. as good or better than customary in malleable iron.

For the manufacture of malleable iron castings, it has been customary to subject the white iron castings, which contain carbon in the combined form, i. e., cementite and pearlite, and which makes the metal hard and brittle, to a suitable heating or annealing treatment, thereby changing the combined carbon to an amorphous free carbon in the form of "temper-carbon", the 15 metal becoming ductile, and known as "malleable cast iron". The annealing treatment usually consists in slowly heating the castings to a temperature of about 1500° F., maintaining them at this temperature for about fifty hours, and then 20 cooling them very slowly. This annealing treatment changes the character of the casting from one having a white silvery crystalline fracture, in which no graphite flakes are visible to the naked eye, to one having a dark gray, soft, velvety appearing fracture, in which the carbon has been 25 precipitated or segregated into rounded masses, leaving little or no carbon combined with the iron. This change takes place at a temperature as low as 1250° F., but occurs more effectively at a temperature of 1350° F. The ordinary commercial 30 temperature range for the treatment is from about 1250° F. to about 1800° F. This change in character of the metal is accompanied by a considerable increase in strength and ductility of the 35 castings, as a result of which they are better able to withstand shock than gray iron castings. Malleable iron castings are accordingly extensively used for agricultural implements, automobiles, railroads, pipe fittings, and hardware.

40 The manufacture of malleable iron castings is, however, very costly, as compared with the manufacture of similar articles by stamping and other fabricating methods, and is moreover attended with difficulties which are not encountered in ordinary stamping practice. In the manufacture 45 of malleable iron castings for automobile brake drums, for example, only the most highly skilled foundries can be relied upon to produce sound castings, with a minimum of rejections. Due to shifting of the patterns in the mold, the 50 sections of the castings are usually heavier than desired in the finished brake drum, and the excess metal is then required to be removed by slow and expensive machining operations. Moreover, certain defects in the castings, which be-

come visible only after machining, such as porosity, shrinks and cold shuts, result in rejections in addition to those resulting from the initial casting operations.

It is among the objects of this invention accordingly, to provide advantageous processes for working iron-carbon alloys, such as white iron castings, by malleabilizing and subsequently rolling, and obtaining products of marked ductility, tensile strength, resistance to corrosion, etc., as contrasted with the initial cast iron. A further object is the production of such modified metal in the form of sheets, strips, bars, tubes, and other shapes, suitable for use as such, or for stamping or fabrication into other products. Other objects and advantages will appear as the description proceeds.

To the accomplishment of the foregoing and related ends, said invention, then, comprises the features hereinafter fully described, and particularly pointed out in the claims, the following description setting forth in detail certain illustrative embodiments of the invention, these being indicative, however, of but a few of the various ways in which the principle of the invention may be applied.

In accordance with my invention, a melt is prepared and is cast into ingots, slabs, or forms as desired. For the composition of the melt some latitude is permissible; however, in general, it is desirable that the carbon be in the amount of from about 1.50 to about 4.00 per cent, silicon from about 0.45 to about 1.75 per cent, manganese below 1 per cent, phosphorus not exceeding 0.225 per cent and desirably under 0.05 per cent and sulphur desirably not exceeding 0.05 per cent. Optionally also, I may add alloying metals, as for instance molybdenum in amounts up to 1 per cent, 0.5 per cent giving in general excellent result; copper in amounts up to 0.6 per cent, etc.

The form and dimensions of the molds may, of course, vary in accordance with the particular further purpose in view. For instance, for strip mill and universal mill work, it is desirable to cast in slabs of about 3 inches thickness, the width being dependent upon the width of ultimate sheet product desired, for instance 12 to 35 inches. For sheet mill rolling slabs of approximately  $\frac{3}{4}$  inch thickness are desirable.

The ingots, slabs or other forms are first malleabilized by heating or annealing them at a temperature or temperatures within the malleabilizing range, i. e., about 1250° F. to about 1800° F., and slowly cooling the same, the purpose of such treatment being to decompose all or a major

part of the combined carbon, causing the carbon to be precipitated in the form of free or temper carbon. The free, massive cementite can best be broken up above about 1400° F., but the excess carbide which exists, when cooled, as pearlite, must be decomposed below this temperature. The length of time necessary to produce the desired malleabilization depends, of course, on the particular analysis of the form and upon the thickness or dimensions of same. In actual practice, the metal is heated to the maximum desired temperature within the graphitizing range and maintained at such temperature for the desired period, after which it is slowly cooled to and below about 1400° F., the cooling period being approximately the same as the heating period. Below about 1250° F., the cooling may be rapid, if desired. A typical annealing cycle is as follows:—

|                          | Hours |
|--------------------------|-------|
| Time heating to 1500° F. | 45    |
| Time holding at 1500° F. | 50    |
| Time cooling             | 60    |

By adding molybdenum to the melt initially, I have found that the annealing or malleabilizing treatment proceeds much more rapidly, and the time may be cut down accordingly. For instance, with stock otherwise requiring about 100 hours heating, with the incorporation of 0.25 per cent of molybdenum in the melt, a heating time of about 36 hours is sufficient to obtain the desired properties.

The aforesaid treatment, as previously stated, results in a malleabilization or precipitation of all or a major part of the combined carbon, the precipitated carbon segregating into rounded masses of temper-carbon distributed throughout a more or less homogeneous matrix of ferrite, or relatively pure iron crystals, and in such a way that the resulting malleable iron is extremely ductile and can be readily rolled or otherwise worked.

The ingots, slabs or other forms thus malleabilized, are then reheated for working or rolling, being first heated to a suitable temperature. The minimum temperature for working or rolling is that, below which rolling is difficult in ordinary rolling mill operations, while the maximum temperature, which I term the critical temperature, and which is dependent on the analysis and other factors, is that which separates the ferritic and austenitic phases of the metal, and above which a resolution of the temper carbon takes place. The rolling, in other words, is conducted while the metal is in the ferritic state. The minimum rolling temperature, in practice, is about 1000° F., while the maximum temperature may be as high as about 1500° F., depending upon the analysis of the metal. Upon examining a section of the metal under the microscope after rolling, it will be observed that the metal comprises a matrix wherein are substantially uniformly distributed and substantially uniformly distorted deposits of free graphite in the form of elongated flakes arranged in approximately parallel relation.

Sheets and other stock produced by the methods which has been outlined can be employed for fabricating if desired, or can be further finished by cold-rolling. A final annealing at a temperature above about 1000° F. is advantageous after cold working, for the purpose of removing rolling strains and to effect recrystallization or equiaxing of the distorted ferrite crystals, such anneal-

ing treatment being similar to that employed for annealing plain low-carbon steel sheets. The temperature range for this final anneal is approximately the same as that for rolling, as hereinbefore described.

Following such annealing treatment, the products are in a condition in which they can be readily stamped or otherwise fabricated into various articles, including a great number which have heretofore been made chiefly in the form of malleable iron castings.

Sheet stock rolled and annealed in accordance with our process has a superior resistance to corrosion as compared with sheet steel, and lends itself particularly to usage in exposed locations. If desired, galvanizing or tinning, etc. may also be applied. On account of the properties of my material, nitriding is especially feasible, and as shaped into desired articles, it may be thus hardened or nitrided by heating with ammonia, along known or practical lines.

It will be understood that various products, in addition to those stated, may be made from the iron-carbon alloy slabs or ingots and that various articles, in addition to those described, may be made from such products. In making tubes, for example, the rolled sheets may be slit into strips (skelp), which are shaped into cylindrical form, welded and annealed; or the slabs or ingots may be rolled directly into skelp, which may be shaped into cylindrical form while hot, welded by well known electric welding processes and annealed, the annealing in either case being optional.

While the term "malleable iron" has been applied to products such as pure or puddled iron, and soft or mild steels, which are admittedly malleable in various degrees and in a greater degree than "malleable cast iron", such designation is entirely improper in the metallurgy of ferrous products, and it is therefore desired to particularly point out that the term "malleable iron" as used and contemplated in the specification and claims is intended to mean "malleable cast iron", which is a product only slightly malleable at ordinary temperatures, but which is tougher than the white cast iron from which it is made. The term "malleable", as employed in this connection is intended to designate a relative condition between white cast iron, which is practically devoid of malleability in its cold state, and "malleable cast iron".

The term "white cast iron", as used in this application, is intended to designate an iron-carbon alloy which is within the range of the melt analysis set forth in the specification. While it usually contains from about 2.00% to about 3.00% carbon and from about .45% to about 1.75% silicon, it may be more generally defined as an iron-carbon alloy containing more than about 2% carbon which solidifies and cools to ordinary temperatures without the formation of graphite.

This application is a continuation-in-part of my applications Serial No. 619,814, filed June 28, 1932, and Serial No. 25,310, filed June 6, 1935.

Other modes of applying the principle of my invention may be employed instead of the one explained, change being made as regards the means and the steps herein disclosed, provided those stated by any of the following claims or their equivalent be employed.

I therefore particularly point out and distinctly claim as my invention:—

1. The process which comprises malleabilizing

5 a white cast iron casting, and thereafter rolling said casting into sheets and other commercially useful products at a temperature not in excess of the lowest temperature at which the temper carbon recombines with the iron.

6 2. The process which comprises malleabilizing a white cast iron casting, and thereafter rolling said casting at a temperature above about 1000° F., but below the lowest temperature at which the 10 temper carbon recombines with the iron.

10 3. The method which comprises rolling into sheets and other commercially useful products malleabilized iron-carbon alloys containing from about 1.50% to about 4.00% carbon.

15 4. The method which comprises rolling malleable cast iron at a temperature of from about 1000° F. to about 1500° F.

20 5. As a new article of manufacture, a sheet-like product formed by rolling a malleabilized iron-carbon alloy containing from about 1.50% to about 4.00% carbon.

25 6. As a new article of manufacture, a sheet-like product formed by rolling malleable cast iron.

7. The method which comprises malleabilizing iron-carbon alloys containing from about 1.50% to about 4.00% carbon and then plastically deforming said malleabilized alloys into products of sheeted and other shapes at a temperature 30 between about 1000° F. and about 1500° F.

8. The method which comprises heat treating white cast iron within the malleabilizing range to precipitate substantially all of the combined carbon as temper carbon and thereafter rolling the same into sheets and other commercially useful products. 5

9. The method which comprises annealing white cast iron to precipitate a major proportion of the carbon as free carbon, thereafter heating said cast iron to a rolling temperature, and rolling said cast iron into sheets and other products. 10

10 10. A metal product comprising rolled graphitic iron having a ferrous matrix wherein are substantially uniformly distributed and substantially uniformly distorted deposits of free graphite 15 in the form of elongated flakes arranged in approximately parallel relation.

11. A metal product comprising rolled graphitic iron having a matrix of ferrite with elongated substantially uniformly distorted deposits of free 20 graphite uniformly distributed therein in parallel relation.

12. The method for making rolled shapes of malleable iron wherein iron as ingots of white iron is subjected to heat treatment in the malleabilizing range and slow cooling to precipitate substantially all of the combined carbon as temper carbon, and is thereafter rolled at temperatures above about 1000° F. 25

NATHAN H. SCHERMER. 30